

## UNITED STATES PATENT OFFICE

MAX BERGMANN, OF DRESDEN, GERMANY

## PROCESS FOR DEPILATING HIDES AND SKINS

No Drawing. Application filed July 27, 1925, Serial No. 46,493, and in Germany February 12, 1925.

The commonly employed means for removing the hair from hides and skins, such as lime-cream and other slackening means, for example:—mixtures of lime-cream and sodium sulfide, lime-cream and arsenic sulfide, lime-cream and sodium hydroxide, sodium sulfide alone, sodium hydroxide alone, sodium hydroxide and enzymes, enzymes alone, or other means for unhauling skins, show the inconvenience that, at the same time as they produce the depilation of the hides and skins, they damage the hair and those portions of the hide or skin from which the hair has been taken off. I now have found that it is possible to avoid this inconvenience and to obtain nevertheless a perfectly satisfactory depilation of the hides and skins if the hides and skins, prior to, the treatment with the commonly used slackening means, or dressing means as lime, lime and sodium sulphide, lime and arsenic sulphide, and the like, are treated with substances which are also able to loosen the hair but do not injure the same. Substances which are in first line suitable for this purpose are inorganic and organic nitrogen bases as ammonia, ethylene diamine, piperidine, pyridine and ureas, and the compounds of said nitrogen bases, as especially the sulphides of such nitrogen bases, and further soluble silicates, these substances being employed separately or mixed with one another. I have found that, if the hides and skins are submitted to a treatment with solutions of the substances mentioned separately or in mixture prior to the treatment with the commonly used unhauling means, the hair or wool and the true skins or the portions of the hides and skins from which the hair has been taken off are not injured at all so that the value of the same is considerably increased. The leather made from skins and hides from which the hair has been taken off in this manner shows a fine, well adhering grain combined with good fullness and a special density without being rigid or brittle.

It has further been found that when the hides and skins have been preliminarily treated with the substances mentioned or

with mixtures thereof the subsequent depilating process proper can be varried out in a fraction of the time which was hitherto necessary for the slackening process by means of lime-cream and the like. When 55 cleansing and working the hides with a mixture of lime-cream and sodium sulphide it is, for instance, possible to reduce by a preliminary treatment of the kind described, the duration of the depilating process from 60 12 hours to half an hour. This effect of the preliminary treatment is very surprising and peculiar. The advantage resides not only in the reduction of duration of the depilating process proper but at the same 65 time in the very good preservation especially of the hair which results from the fact that the lime-cream or the like which impairs the hair acts upon the skin and hair only for a very short time. If the hides and skins prior 70 to the action of one of the commonly used slackening means are treated with solutions of ammonium sulphide or other ammonia derivatives alone or in mixture with soluble silicates, so weak concentrations of these 75 solutions can be used that they do not cause a serious loosening of the hair, and only in combination with one of the commonly used, subsequently applied slackening means they effect sufficient depilation. A similar, al- 80 though smaller effect is obtained if the soluble silicates are applied alone. But these products must always be applied prior to the tanning process proper if the desired 85 action upon the true skin shall occur.

*Examples of application*

1. For unhauling or depilating a set of sheepskins or fleeces they are brought, after having been well soaked, into a solution 90 which contains for one cubicmeter of water 10 liters of a technical solution of ammonium sulphide with a content of 10%  $(\text{NH}_4)_2\text{S}$ , and they are left in this solution for one day. The skins are then put in an aqueous liquor 95 which contains 0,25 kilo of sodium sulphide for each cubicmeter of liquid and lime in such a quantity that it will be well in excess of saturation of the liquid. After one hour the skins will release the hair, quite 100

readily, and skins and hair are absolutely uninjured.

Instead of the indicated liquid for the preliminary treatment a solution may be used which contains for one cubicmeter of

water 10 liters of 25% ammonia. Instead of the liquid containing lime and sodium sulphide, an aqueous liquor containing 15 kilos of lime and 1.75 kilos of arsenic sulphide for each cubicmeter may be used for the unhairing process or also any one of the other commonly used unhairing means may be employed.

2. For unhairing a set of calfskins they are brought into a solution which contains for one cubicmeter of water 10 liters of a technical ammonium sulphide solution with a content of 10%  $(\text{NH}_4)_2\text{S}$  and 10 liters of commercial water-glass solution of 38° to 20° Bé. So much of the liquid is used that the skins are well covered. After one day the skins are washed for three hours in water which has to be renewed several times and they are then brought into an aqueous liquid mixture carrying 10% of lime and 1% of crystallized sodium sulphide. After one day, or at the utmost two days (according to the thickness of the skins), they will release the hair readily, hair and skins being quite uninjured, and the leather obtained after tanning possesses a well adhering grain and great density.

For other hides and skins the process must be modified accordingly although it remains principally the same.

Instead of ammonia or ammonia derivatives, suitable organic nitrogen bases and derivatives of the same may be used, as for instance ethylenediamine, piperidine, pyridine, urea substances and the like, or other mildly acting hair-loosening means either alone or in mixture.

Having now particularly described and ascertained the nature of my said invention, I declare that what I claim is:

1. A process for unhairing skins and hides which comprises firstly treating the skins and hides with a watery solution containing a nitrogen base readily soluble in water while giving it an alkaline reaction, and then with an alkaline unhairing means.

2. A process for unhairing skins and hides which comprises firstly treating the skins and hides with a soluble compound containing a nitrogen base readily soluble in water while giving it an alkaline reaction and then with an alkaline unhairing means.

3. A process for unhairing skins and hides which comprises treating the skins and hides with a mixture of compounds containing a nitrogen base readily soluble in water while giving it an alkaline reaction and with an alkaline unhairing means.

4. A process for unhairing skins and hides which comprises firstly treating the skins

and hides with a basic derivative of a nitrogen base readily soluble in water while giving it an alkaline reaction and then with an alkaline unhairing means.

5. A process for unhairing skins and hides which comprises firstly treating the skins and hides with a basic derivative of ammonia which is readily soluble in water while giving it an alkaline reaction and then with an alkaline unhairing means.

6. A process for unhairing skins and hides which comprises firstly treating the skins and hides with a mixture containing a derivative of a nitrogen base which is readily soluble in water while giving it an alkaline reaction, and an alkali metal silicate and thereafter with an alkaline unhairing means.

7. A process for unhairing skins and hides which comprises firstly treating the skins and hides with a mixture of ammonium sulphide and an alkali metal silicate and thereafter with an alkaline unhairing means.

8. A process for unhairing skins and hides which comprises treating the skins and hides with a watery solution containing a nitrogen base readily soluble in water while giving it an alkaline reaction and with an alkaline unhairing means.

9. A process for unhairing skins and hides which comprises treating skins and hides with ammonium sulphide and an alkaline unhairing means.

10. A process for unhairing skins and hides which comprises treating the skins and hides with a watery solution of a basic derivative of ammonia readily soluble in water while giving it an alkaline reaction, a part at least of the hydrogen of which is substituted by a hydrocarbon group, and with an alkaline unhairing means.

11. A process for unhairing skins and hides which comprises treating skins and hides with ammonium sulphide, and with a chemical slackening means containing lime.

12. A process for unhairing skins and hides which comprises firstly treating the skins and hides with a mixture of ammonium sulphide and an alkali metal silicate, and thereafter with a chemical slackening means containing lime.

In testimony whereof I have hereunto set my hand.

DR. MAX BERGMANN.

120

125

130